

## UNITED STATES PATENT OFFICE

2,003,148

METHOD AND MEANS FOR COMPOUNDING  
FLAME AND WATERPROOFING COMPOSI-  
TIONS FOR AQUEOUS CELLULOSIC MEDIAFrederick W. Hochstetter, Pittsburgh, Pa., as-  
signor to Treedsdale Laboratories, Inc., a cor-  
poration of Delaware

Application March 23, 1933, Serial No. 662,291

2 Claims. (Cl. 134—78.6)

This invention concerns the flame and water-proofing of aqueous cellulosic media and to a composition of matter therefor together with the method of making the same.

As pointed out in my copending application 651,363, filed January 12, 1933 for Flame-proofing composition of matter and process for making the same, it has heretofore been considered commercially impossible to render aqueous cellulosic media both flame and water-proof. If the water-proofing compound was applied first its effectiveness was destroyed by the application of the flame-proofing composition, and vice versa, and in addition there was no single composition known which would render such media both flame and water-proof.

One of the objects of the present invention is to overcome the above mutually destructive effects of utilizing separate mutually hostile flame and water-proofing compositions and to provide a single composition which will accomplish both results effectively and practicably.

Another object of my invention resides in the method of compounding a single composition which will render aqueous cellulosic media both flame and water-proof as well as a method for making such composition.

A further object resides in compounding certain relative quantities under controlled conditions.

A still further object resides in the process and arrangement of apparatus for compounding certain specified constituents in certain relative proportions under controlled conditions in a certain order and in applying the same to the medium so as to secure the greatest effect therefrom.

Other and further objects and advantages will be understood by those skilled in the art or will be apparent or will be pointed out hereinafter.

In the accompanying drawing the figure illustrates a more or less schematic arrangement for compounding the composition of matter and for applying it to the medium as will be hereinafter more fully described.

In the upper left-hand corner of the figure of the drawing are a number of containers or vessels in which I preliminarily provide the various solutions from which the present composition of matter may be made. Reading from left to right these containers are designated to contain alum solution, boric acid solution, ammonium carbonate solution, ammonium sulphate solution, aqueous colloid solution, ammonium chloride solution, boric acid solution, borax solution, and soap solution. It is to be understood at the out-

set that this arrangement is variable according to circumstances, but in general the solutions are more or less so arranged in the receptacles that certain groups of them can be discharged into common or predetermined receptacles or tanks. As shown each solution container 10 is provided with a lower discharge pipe 11, each such discharge pipe being provided with a suitable valve 12 for opening or closing the pipe 11 or for controlling the rate of flow therethrough. It will be noted that the aqueous colloid solution container has two such discharge pipes as it may be desired to discharge part of the solution into different tanks or if such is not the case, either pipe 11 may be used while the other is shut off.

As shown in the drawing further these discharge pipes 11 are so directed as to discharge into a selected one of a number of tanks indicated by the numeral 13, two such tanks being shown although any required or desired number may be used. Each such tank 13 is provided with a suitable temperature indicating device 14 and with any necessary or desired gauge member 15. Predetermined amounts from predetermined receptacles are discharged into the selected tank 13 as will hereinafter more in detail be pointed out.

Each of tanks 13 in turn is provided with a discharge 16 having a suitable valve 17 therein, and, as shown these discharge pipes lead to a larger mixing tank 18, likewise provided with a temperature indicating device 19. In this tank the final composition is brought to condition and from such tank the composition when finished may either be directed directly to the treating tank 24, or if a succeeding portion of material is being finished in tank 18, previously completed composition may in the meanwhile be held in intermediate tank 21, also provided with a temperature indicating device 22, and from which tank the finished solution can be fed as needed to treating tank 24 by way of suitable pipes and valves as will be understood.

The method schematically outlined above comprises in detail the following steps and operations substantially in the order named except as otherwise pointed out.

First, for example, I heat five gallons of water to about 120° F. and to the same I add in the order named 48 ounces of ammonium sulphate, 16 ounces of ammonium carbonate, 20 ounces of boric acid and 16 ounces of borax. Upon adding the ammonium sulphate, stirring is carried out to ensure complete dissolution thereof in the water. The ammonium carbonate is added incre-

mentally under constant stirring, care being taken to prevent violent effervescence which may occur. The boric acid previously dissolved in one gallon of boiling water is not added until effervescence has ceased, and, after thoroughly admixing these three, the borax is then added and thoroughly mixed by stirring or the like. Next, I add under constant stirring to the foregoing, 16 ounces of starch such as arrow-root starch which has been previously cooked to about 1° Baumé. I then dissolve 6 ounces of any suitable soap in one gallon of water and bring this up to the boiling point by heating, whereupon it is added to the foregoing ingredients. An emulsification takes place upon the addition of the soap solution and when complete emulsification has taken place the temperature is reduced to about 110° F. and the composition digested for two hours, thereby forming a first composition. I heat five gallons of water to the boiling point and dissolve therein five pounds of ammonium chloride, 3 pounds of boric acid and one pound of borax in the order named, and each succeeding material is added only after the preceding is entirely dissolved. After stirring this thoroughly I dissolve 2 pounds of soft gelatin and 2 gallons of water and heat to 200° F. under constant stirring, to which 400 c. c. of glycerin or its equivalent may be added if a flexible medium is desired. I thoroughly stir the gelatin solution and then mix it with the ammonium chloride—boric acid—borax solution under constant stirring for about thirty minutes and then the same is digested for about one hour at about 140° F.; I dissolve 3 ounces of any suitable soap, such as sodium resinate, stearic acid or sodium stearate, in one gallon of water, heat to the boiling point and add 8 ounces of dextrine, stirring such constantly to ensure uniformity, and then, adding such to the ammonium chloride—boric acid—borax—gelatin solution, thereby forming a second composition.

To form my third composition I heat one gallon of water to the boiling point and add thereto 15 ounces of soap bark (tannin). The soap bark is dissolved and if necessary the solution is filtered to remove undissolved matter.

To form my fourth composition I dissolve 32 ounces of alum—preferably neutral alum—in 2 gallons of cold water.

Each of these four compositions are digested additionally for a period of about four hours, stirring occasionally or from time to time to prevent the settling out at the bottom of colloidal matter. After each of the four compositions is thus compounded and treated I finally combine them in a common vessel in the order one, two, four, three. In other words, the first two compositions are added in order to the vessel and then the fourth composition is added, the third composition being reserved until last and being added under vigorous constant stirring.

If the ingredients of the above-mentioned compositions are designated or expressed as parts, since one gallon fluid measure is equivalent to 128 fluid ounces, and one pound avoirdupois is equivalent to 16 avoirdupois ounces, and one cubic centimeter is equivalent to .03381 fluid ounces, by way of example, the first composition includes 640 parts of water at 120° F. to which is added 48 parts of ammonium sulphate, 16 parts of ammonium carbonate, 20 parts of boric acid, and 16 parts of borax. The boric acid is previously dissolved in 128 parts of water, 16 parts of starch

are added and 6 parts of soap are dissolved in 128 parts of water.

In the second composition, the 5 gallons of water may be designated as 640 parts, the 5 pounds of ammonium chloride as 80 parts, the 3 pounds of boric acid as 48 parts, the 1 pound of borax as 16 parts, the 2 pounds of solid gelatine as 32 parts, the 2 gallons of water as 256 parts, the 400 c. c. of glycerine as 13½ parts, the 3 ounces of suitable soap as 3 parts, the 1 gallon of water as 128 parts, and the 8 ounces of dextrine as 8 parts.

In the third composition, the 1 gallon of water may be represented as 128-parts and the 15 ounces of soap bark as 15 parts.

In the fourth composition, alum may be represented as 32 parts and the water as 256 parts.

It should be noted that when I refer to a fluid such as water as including so many parts, that I have reference to fluid parts, and further, when referring to a substance such as alum, soap, etc., that I refer to avoirdupois parts.

In certain cases where it is impractical or inconvenient I may modify the above method by dissolving each constituent above named separately in water, if water-soluble, to form stock solution. These stock solutions would then be combined in the proper proportions and at the proper temperatures and under the proper conditions above set forth before being used.

In applying the composition of the present invention to the medium to be flame and water-proofed, it may be any suitable aqueous cellulosic medium or any suitable textile or fabric material or an equivalent or derivative thereof. I proceed in a typical case as shown in the right-hand portion of the figure of the drawing. A suitable roll of the material to be treated 30 is revolvably mounted as on a roller 31 journaled in standards 32 whereby the material can be readily unrolled. It passes first by way of suitably constructed idler and/or tension rolls 33 through the treating tank 24 to which is fed my present composition of matter as will be understood from the drawing. The length of the tank is such that the material will be subjected to the composition for the desired length of time after which the material emerges from the tank and passes more or less vertically upwardly between the rollers 34 which act as squeeze rollers thus eliminating excess composition from the material. These squeeze rollers may be so arranged in relation to the treating tank 24 that the excess composition may either drop back to the tank or be otherwise collected and saved for re-use. From squeeze rollers 34 the material then passes through tension rollers 35 whence it is guided as by means of short endless belts 36 mounted on rollers 37 into the interior or vaporizing chamber 38 of treating chamber 60. Belts 36 may be synchronized perforated rubber belts and the right hand set of rolls may be perforated, hollow, and connected to a vacuum or suction connected as hereinafter pointed out in connection with members 40 and 41.

In vaporizing chamber 38 air, heated or otherwise, is caused to pass over, through and around the treated material so as to effect almost instantaneous vaporization of excess composition and to complete a substantial drying of the material. Such vaporizing air may be suitably generated as by a supply blower or fan 61 which creates a blast of air through conduit 62, since it is connected as by a suitable fitting 63 into the vaporizing chamber.

By way of guide rolls 39 mounted in the exit side of the vaporizing chamber the material is

caused to pass over a rubber perforated belt 40 mounted in endless fashion on the rolls 41. One of such rolls 41 is shown as hollow and provided with perforations 42 and connected to this hollow 5 roll by means of a suitable connecting pipe 43 is an exhaust or vacuum pump or fan 44 which results in a sucking of air through the rubber perforated belt 40, thus holding the material in contact with the rubber belt, and, further drying 10 the material which may be additionally assisted by a hood 64 of frusto-conical shape connected into conduit 62 and having, if desired, a thermostatically controlled stem or electrical means for warming or heating the air passing through said 15 hood. As shown such is represented by an electrical resistance coil 65 and it is clear that the hood itself directs air onto the rubber belt and the medium thereon. Roller 45 may be provided for any suitable purpose such as maintaining close 20 contact between the various elements at the perforated roll. While the rubber belt and its rolls have been shown as located within a chamber 46, this chamber may or may not be used and is only illustrative.

25 From the perforated roll the material passes by way of suitable idler or guide rolls 47 to a festooning machine indicated by the numeral 48 and consisting mainly of a framework having cross bars 49 on which are journalled suitable 30 rolls 50, so that the material passing therethrough can be given a relatively long and tortuous path for completing the drying and for ensuring a straight unwrinkled product. Analogous to the frusto-conical hood 64 is a second 35 similar hood 66 bearing the same relative relationship to the festooning machine 48 as the first hood bears to the perforated rubber belt and its rolls.

From the festooning machine the material 40 passes through calender rollers 51 and is finally re-wound on roller 52 journalled in standards 53 to form a roll 54 of finished material. I have, therefore, disclosed a single composition of matter which consists of a more or less complex 45 solution together with a means for making the same which is adapted efficiently to render media of the nature explained both flame and water-proof at one and the same time. Upon compounding such a composition and then applying it to the medium or material to be flame 50 and water-proofed and then drying the same after the application of the composition, I find that I can accomplish in a single and relatively simple process a finished commercial article 55 which is non-flammable and water-proof.

It is clear that the above is intended more in an illustrative than in a limitative manner and I may make suitable or desired modifications, substitutions, additions or omissions without departing from the spirit and scope of the invention, particularly as designed by the subjoined 60 claims. For example, I am not strictly limited to the precise constituents set forth, but such is on the contrary subject to some considerable 65 variation. In a particular case constituents are chosen which will have the desired effect upon the particular medium and which will contain nothing deleterious to that medium which, incidentally, has been one of the serious difficulties 70 with previously contemplated compositions. I may also in similar manner vary the concentrations or amounts of the constituents depending again upon the particular medium being treated and the degree of resistance to flame and water 75 which is to be imparted. Other and further

variations will be understood by those familiar with the compounding of chemicals and the treating of various media therewith.

In setting forth the foregoing it is further to be understood that where I specify certain chemicals I am not limited to precisely such but I thereby intend to include their equivalents or substitutes, capable of producing the intended results.

What I claim as new and desire to secure by Letters Patent is:

1. A method of flame and water-proofing aqueous cellulose media comprising carrying out the following steps in substantially the relative proportions indicated as follows: heating 640 parts of water to 120° F., adding 48 parts of ammonium sulphate and stirring until completely dissolved, adding 16 parts of ammonium carbonate incrementally under constant stirring until effervescence ceases, adding 20 parts of boric acid previously dissolved in 128 parts of boiling water, adding 16 parts of borax and thoroughly mixing, adding 16 parts of starch previously cooked to about 1° Baumé and thoroughly mixing in the same under constant stirring; dissolving 6 parts of suitable soap in 128 parts of water and bringing it to the boiling point, thereafter adding the same to the previously compounded materials, bringing about emulsification of the whole, and then, lowering the temperature to about 110° F. and digesting for about 2 hours, thereby forming a first composition; bringing 640 parts of water to the boiling point and dissolving therein 80 parts of ammonium chloride, 48 parts of boric acid and 16 parts of borax in the order named and each after the preceding has been completely dissolved, stirring the same thoroughly after all three have been added and dissolved, separately dissolving 32 parts of soft gelatine in 256 parts of water and heating to about 200° F. under constant stirring, and thereafter, optionally adding thereto 13½ parts of glycerine, stirring thoroughly, and then, adding the same to the ammonium chloride—boric acid—borax solution under constant stirring for about 30 minutes, and then digesting for about one hour at about 140° F.; dissolving 3 parts of suitable soap in 128 parts of water, heating to boiling and adding 8 parts of dextrine, stirring such constantly to ensure uniformity and then adding such to the ammonium chloride—boric acid—borax—gelatine solution, thereby forming a second composition; bringing 128 parts of water to the boiling point, dissolving therein 15 parts of soap bark and filtering, thereby forming a third composition; dissolving 32 parts of alum in 256 parts of water as a fourth composition; digesting each of the four compositions for about 4 hours while stirring from time to time; combining the first, second and fourth compositions in a common vessel and then adding the third composition under vigorous stirring, suitably applying the whole to the medium and then drying the same.

2. A method of compounding a composition of matter for flame and water-proofing aqueous cellulose media and their derivatives comprising heating 640 parts of water to 120° F., adding 48 parts of ammonium sulphate and stirring until completely dissolved, adding 16 parts of ammonium carbonate incrementally under constant stirring until effervescence ceases, adding 20 parts of boric acid previously dissolved in 128 parts of boiling water, adding 16 parts of borax

and thoroughly mixing, adding 16 parts of starch previously cooked to about 1° Baumé and thoroughly mixing in the same under constant stirring; dissolving 6 parts of suitable soap in 128 parts of water and bringing it to the boiling point, thereafter adding the same to the previously compounded materials, bringing about emulsification of the whole and then lowering the temperature to about 110° F. and digesting for about 2 hours thereby forming a first composition; bringing 640 parts of water to the boiling point and dissolving therein 80 parts of ammonium chloride, 48 parts of boric acid and 16 parts of borax in the order named, and each after the preceding has been completely dissolved, stirring the same thoroughly after all three have been added and dissolved, separately dissolving 32 parts of soft gelatine in 256 parts of water and heating to about 200° F. under constant stirring and thereafter optionally adding thereto 13½ parts of glycerine, stirring thoroughly and then adding the same to the ammonium chloride-boric acid-borax solution under constant stirring for about 30 minutes and then digesting for about one hour at about 140° F.; dissolving 3 parts of suitable soap in 128 parts of water, heating to boiling and adding 8 parts of dextrine, stirring such constantly to ensure uniformity and then adding such to the ammonium chloride-boric acid-borax-gelatine solution, thereby forming a second composition; bringing 128 parts of water to the boiling point, dissolving therein 15 parts of soap bark and filtering, thereby forming a third composition; dissolving 32 parts of alum in 256 parts of water as a fourth composition; digesting each of the four compositions for about 4 hours while stirring from time to time; combining the first, second and fourth compositions in a common vessel and then adding the third composition under vigorous stirring.

FREDERICK W. HOCHSTETTER.

5

10

15

20